

1

2,820,723

## INHIBITION OF CORROSION OF PHOSPHATED METAL SURFACES

William M. Le Suer, Cleveland, Ohio, assignor to The Lubrizol Corporation, Wickliffe, Ohio, a corporation of Ohio

No Drawing Application January 17, 1957  
Serial No. 634,627

11 Claims. (Cl. 117—127)

This invention relates to a process for the inhibition of corrosion of metal surfaces and in particular to a process which is particularly useful for the inhibition of corrosion of ferrous metal surfaces.

The corrosion of metal surfaces is of obvious economic significance in many industrial applications, and as a consequence the inhibition of such corrosion is a matter of prime consideration in such applications. It is a particular significance to users of steel and other ferrous alloys. The corrosion of such ferrous metal alloys is largely a matter of rust formation which in turn involves the overall conversion of the free metal to its oxide.

The theory which best explains such oxidation of ferrous metal surfaces postulates the essential presence both of water and oxygen. Even minute traces of moisture are sufficient, according to this theory, to induce the dissolution of iron therein and the formation of ferrous hydroxide until the water becomes saturated with ferrous ions. The presence of oxygen causes oxidation of the resulting ferrous hydroxide to ferric hydroxide which then settles out of solution and is ultimately converted to ferric oxide or rust.

The above sequence of reactions can be prevented, or at least in large measure inhibited, by relatively impermeable coatings which have the effect of excluding either or both moisture and oxygen from contact with the ferrous metal surfaces. Such coatings are, of course, subject to abrasion and other causes of physical deformation and to the extent that these coatings are penetrated or otherwise destroyed by such influences they are ineffective for the purpose desired. It is important that such coatings provide complete protection of all of the ferrous metal surfaces. If there is any portion of such a surface which is not so protected, regardless of how small the unprotected surface may be, the degree of protection afforded is considerably less than desirable. A satisfactory corrosion-inhibiting coating, then, must have the ability to resist substantial deformation upon impact, abrasion, etc. so that a uniform and complete film of protection is maintained in the face of such adverse influences.

It is accordingly a principal object of this invention to provide protection from corrosion for metal surfaces.

It is another object of this invention to provide protection from the formation of rust on ferrous metal surfaces.

Other objects will be apparent from the ensuing description.

These objects are achieved by the process of inhibiting corrosion of phosphated metal surfaces which comprises applying to said surfaces a film of a product prepared by the process which comprises the reaction of

(a) A zinc salt of a phosphorodithioic acid with  
(b) An approximately equivalent amount of an organic epoxide containing at least 4 aliphatic carbon atoms.

The zinc salt of a phosphorodithioic acid which may be used as reactant (a) in the preparation of the above-described rust-inhibiting agent is easily prepared merely

2

by reaction of zinc oxide with the appropriate phosphorodithioic acid.

The phosphorodithioic acid likewise is conveniently prepared by reaction of phosphorus pentasulfide with an alcohol or phenol, or with a mixture of alcohols or phenols. It has been shown, and is disclosed in detail in copending application, Serial No. 612,597, filed September 28, 1956, that the polyvalent metal salts of phosphorodithioic acids prepared from a mixture of a monohydric and a polyhydric alcohol have superior rust-inhibiting properties with respect to the corresponding polyvalent metal salts of "simple" phosphorodithioic acids, i. e., those prepared by the reaction of phosphorus pentasulfide with a single alcohol, either monohydric or polyhydric.

The compositions of this invention are derivable from phosphorodithioic acids of either of the above types. In some particular instances those which are prepared from zinc salts of "simple" phosphorodithioic acids are preferable to those prepared from zinc salts of mixed phosphorodithioic acids, although for most applications the reaction products prepared from the zinc salts of mixed phosphorodithioic acids are preferable.

The terms "simple" and "mixed" refer, of course, to phosphorodithioic acids prepared from in the first case a single alcohol, and in the second case from a mixture of a monohydric and a polyhydric alcohol.

Phosphorodithioic acids may be represented by the structural formula:



in which R and R' are organic radicals attached to the oxygen atoms through carbon atoms. The reaction of alcohols with phosphorus pentasulfide yields phosphorodithioic acids in which R and R' are attached to the oxygen through aliphatic carbon atoms. Correspondingly the same reaction with phenolic compounds yields phosphorodithioic acids in which R and R' are attached to these oxygens through benzenoid carbon atoms. Although it is more desirable for the purposes of this invention to employ phosphorodithioic acids in which R and R' are aliphatic this preference is predicated largely on reasons of economy and in the absence of such reasons the aromatic phosphorodithioic acids would be satisfactory in many instances. Particularly useful phosphorodithioic acids are available from such alcohols as butyl, hexyl, octyl, and mixtures of these alcohols with ethylene glycol, propylene glycol, dipropylene glycol and glycerol. Particularly preferred phosphorodithioic acids may be prepared by reaction of phosphorus pentasulfide with mixtures of isoctyl alcohol and 1,2-propylene glycol, isoctyl alcohol and dipropylene glycol, isoctyl alcohol and ethylene glycol.

For a more detailed description of the mixed phosphorodithioic acids which may be used in the preparation of the zinc salt reactants of the process of this invention, reference may be had to the disclosure of the above-identified copending application.

The epoxide reactant (b) includes, as stated previously, only those epoxides which contain within their molecular structure at least 4 aliphatic carbon atoms. It has been observed that the products obtained from the lower molecular weight epoxides, while markedly effective in acting to prevent the corrosion of metal surfaces, are not as effective as those products which result from the use of the higher molecular weight epoxides in the herein-described process. Thus the lowest molecular weight epoxide which has been found to be effective in the preparation of satisfactory anti-corrosion agents is butene oxide,

The use of this epoxide in the herein-described process results in the formation of products which are useful as a surface film to protect metal surfaces in corrosive environments. The use, however, of higher molecular weight epoxides in the process particularly those aliphatic epoxides containing 12-20 carbon atoms per epoxy group, results in products which provide an even greater degree of protection in such environments. For this reason such epoxides as dodecene oxide, hexadecene oxide, butyl oleate oxide, methyl oleate oxide, epoxidized soy bean oil etc. are preferred epoxides for use in this reaction.

The process conditions by which the corrosion-preventive agents of this invention may be prepared include a temperature within the range of 20-200° C. In most cases the reaction is exothermic so that it may in such cases be carried out at relatively low temperatures, viz., in the range of 20-80° C. In other cases where the reaction is not exothermic or where the molecular weight of the reactants is great enough to minimize the thermal effects of an exothermic reaction it is desirable to maintain a higher temperature, viz., in the range of 80-200° C. In most cases, however, a temperature within the range of 50-100° C. is preferred.

The chemical reaction involved in the process of this invention is not understood. The product which results appears not to be a salt, but further than this there is no information available which allows an identification of the molecular structure of the product. For this reason it is necessary to define the product in terms of its process of preparation. In this connection, however, it has been noted that in those cases which involve an exothermic reaction, the exothermic reaction appears to involve at least about two moles of epoxide per mole of zinc phosphorodithioate. Thus one mole of a zinc phosphorodithioate will react exothermically with two moles of certain epoxides. The product of the reaction contains phosphorus, sulfur, and zinc in essentially the same ratio as these elements appear in the zinc phosphorodithioate starting material.

Particular details of the process by which the corrosion-inhibiting agents of this invention may be prepared are illustrated in the following examples.

#### Example 1

A zinc salt of a phosphorodithioic acid was prepared by the reaction of phosphorus pentasulfide with 4 moles of a mixture of equivalent amounts of isoctyl alcohol and propylene glycol, followed by neutralization of the resulting acidic product with zinc oxide. To 670 grams (1.0 equivalent) of this zinc salt there was added at 60-70° C. 76 grams (1.0 equivalent) of butylene oxide. The ensuing reaction was exothermic so that the indicated temperature range was maintained by portionwise addition of the butylene oxide throughout a 30-minute period. The mixture was heated at 67-70° C. for an additional 2 hours, then flushed with a stream of nitrogen at room temperature for 3 hours. The resulting product was a clear liquid having the following analyses:

|    | Percent |
|----|---------|
| P  | 4.6     |
| S  | 9.2     |
| Zn | 4.6     |

#### Example 2

To 1340 grams (2.0 equivalents) of the zinc phosphorodithioate prepared as in Example 1 there was added at 70-72° C. 880 grams (2.0 equivalents) of butyl epoxy stearate (prepared by the epoxidation of butyl oleate). Although the reaction did not appear to be exothermic the butyl epoxy stearate was added portionwise over a period of 2 hours and 45 minutes, the temperature being maintained at 70-72° C. throughout this addition and for an additional 3 hours. The product was filtered through

a siliceous filter aid to yield a clear, light yellow liquid having the following analyses:

|    | Percent |
|----|---------|
| P  | 3.0     |
| S  | 6.0     |
| Zn | 3.0     |

#### Example 3

The zinc salt of a phosphorodithioic acid was prepared by the reaction of phosphorus pentasulfide with a 1:3 (equivalents) mixture of isoctyl alcohol and propylene glycol, followed by reaction of the acidic product with zinc oxide. To 673 grams (1.0 equivalent) of this zinc salt, at 60-70° C., there was added 72 grams (1.0 equivalent) of butylene oxide over a period of 45 minutes. The reaction was slightly exothermic. The mixture was heated for an additional 2 hours at 60-70° C. Nitrogen was bubbled through the mixture at room temperature for 3 hours resulting in a clear liquid having the following analyses:

|    | Percent |
|----|---------|
| P  | 3.7     |
| S  | 7.7     |
| Zn | 5.8     |

#### Example 4

To 1346 grams (2.0 equivalents) of the zinc salt prepared as in Example 3 there was added at 70° C. 880 grams (2.0 equivalents) of butyl epoxy stearate over a period of 80 minutes. When the exothermic reaction had subsided the product mixture was heated for an additional 2 hours at 70-75° then filtered. The filtrate showed the following analyses:

|    | Percent |
|----|---------|
| P  | 3.6     |
| S  | 7.0     |
| Zn | 3.3     |

#### Example 5

The zinc salt of a phosphorodithioic acid was prepared by the reaction of phosphorus pentasulfide with a 1:1 (equivalents) mixture of isoctyl alcohol and ethylene glycol, followed by reaction of the acidic product with zinc oxide. To a solution of 1034 grams of this salt (1.5 equivalents) in 1333 grams of toluene there was added portionwise over a period of 3 hours 276 grams (1.5 equivalents) of dodecene oxide. The temperature was maintained at 80-90° C. throughout the addition and for one hour thereafter. The resulting product showed the following analyses:

|    | Percent |
|----|---------|
| P  | 3.9     |
| S  | 2.1     |
| Zn | 2.1     |

#### Example 6

To 530 grams (0.82 equivalent) of the zinc salt prepared as in Example 5 there was added dropwise over a period of 2 hours 170 grams (0.82 equivalent) of epoxy-propyl amyl sulfide (prepared by the reaction of amyl mercaptan with chloropropylene oxide). The temperature was maintained at 90-100° C. throughout the addition and for 2 hours thereafter. The resulting product had the following analyses:

|    | Percent |
|----|---------|
| P  | 11.4    |
| S  | 3.6     |
| Zn | 4.0     |

#### Example 7

To 700 grams (2.2 equivalents) of zinc di-n-butyl phosphorodithioate there was added dropwise over a period of 4 hours 330 grams (2.2 equivalents) of phenoxy-propylene oxide. The temperature was maintained at 60-80° C. throughout the addition and for an additional

2 hours. The resulting product showed the following analyses:

|    | Percent |
|----|---------|
| P  | 16.1    |
| S  | 7.5     |
| Zn | 7.5     |

As indicated earlier the process of this invention is concerned with the application of products of the type illustrated in the above examples to a phosphated metal surface. The term "phosphated" refers to a treatment by which a metal surface is rendered relatively inactive to corrosion by moisture, air, etc. Such "phosphating" treatments are well known and are described in U. S. Patents 1,206,075; 1,247,668; 1,305,331; 1,485,025; 1,610,362; 1,980,518; and 2,001,754. They generally comprise immersing the metal surface to be treated in a hot aqueous solution of phosphoric acid and/or phosphate salts, which solution also contains one or more inorganic salts such as zinc nitrate, calcium nitrate, copper sulfate, etc. The hot solution acts chemically on the metal surface to form an adherent crystalline deposit of bluish-grey to dark blue color. In instances of mildly corrosive environments such phosphating treatment may provide a satisfactory corrosion-proof result. For the purposes of this invention, however, a mere phosphating treatment is not sufficient. Phosphating serves to provide an initial passivation of the metal surface which must be reinforced with the coating composition described herein.

The following is presented to illustrate a practice of the invention and the advantages secured thereby: 3" x 3" phosphated steel panels, the edges of which have previously been painted with an air-drying enamel, are dipped into a solution of the zinc phosphorodithioate-organic epoxide reaction product in any suitable volatile organic solvent such as, e. g., benzene, toluene, xylene, methyl-ethyl ketone, butyl alcohol, etc. The purpose of the enamel edge-coating is to improve the reproducibility of the corrosion test to be carried out. The panels are withdrawn from the solution at a specified rate so as to insure a uniformly thick film and the solvent is allowed to evaporate. Then the panels are placed in an enclosed cabinet which contains a 5% aqueous solution of sodium chloride at 95° C. This sodium chloride solution is agitated by means of a vigorous stream of air bubbled through the solution so as to produce a corrosive salt-steam atmosphere in the cabinet. The resistance of the panels to corrosion is measured in terms of the time required to produce a single rust spot on the panel in this atmosphere. It is apparent that the degree of protection from corrosion will be related to the thickness of the film which is deposited upon the metal surface, so that any numerical measure of protection from corrosion must take into account this factor of film thickness. Accordingly, the thickness of the film is expressed in terms of milligrams (of film) per square foot (of metal surface area). The use of this expression allows an evaluation of the effectiveness of the corrosion-preventing films of this invention in terms of "hours (of rust-free exposure in a salt-steam atmosphere), per milligrams (of film), per square foot (of metal surface area). In order to facilitate the comparison of these values for different films the "salt-fog life" described above has been expressed as "hours/250 mg./ft.<sup>2</sup>."

The effectiveness of the compositions of this invention as film-forming inhibitors of corrosion is shown by the following table in which each "salt-fog life" represents an average of results from six separate phosphated steel panels containing films of different thicknesses. Each of the steel panels was first "phosphated" by immersion for 6 minutes in a solution containing 1.6 moles of phosphoric acid ( $H_3PO_4$ ), 0.4 mole of mono-ammonium phosphate ( $NH_4H_2PO_4$ ), 1 mole of zinc nitrate ( $Zn(NO_3)_2$ ), and 1 mole of calcium nitrate ( $Ca(NO_3)_2$ ) at 180-190° F. The panels are removed, rinsed with hot

water and then with dilute chromic acid (0.5 grams/liter) at 180-190° F.

| Percent | Example No. | Rust-proofing composition                                                                                                                                                         | Salt-fog life (hours/250 mg./ft. <sup>2</sup> ) |
|---------|-------------|-----------------------------------------------------------------------------------------------------------------------------------------------------------------------------------|-------------------------------------------------|
| 16.1    | 5           | None                                                                                                                                                                              | 6                                               |
| 7.5     | 8           | Product of Example 1                                                                                                                                                              | 214                                             |
| 7.5     | 9           | Product of Example 2                                                                                                                                                              | 530                                             |
|         | 10          | Product of Example 3                                                                                                                                                              | 88                                              |
|         | 11          | Product of Example 4                                                                                                                                                              | 493                                             |
|         | 12          | Product of Example 5                                                                                                                                                              | 845                                             |
|         | 13          | Product of Example 6                                                                                                                                                              | 397                                             |
|         | 14          | Product of Example 7                                                                                                                                                              | 265                                             |
|         | 15          | A product prepared as in Example 2 except that the phosphorodithioic acid is prepared from a mixture of 35 molar parts of isoctyl alcohol and 65 molar parts of propylene glycol. | 513                                             |
|         | 16          | A product prepared as in Example 1 except that the phosphorodithioic acid is prepared as in Example 16.                                                                           | 179                                             |
|         | 17          | A product prepared as in Example 5 except that the glycol used in the preparation of the phosphorodithioic acid is dipropylene glycol.                                            | 394                                             |
|         | 18          | A product prepared as in Example 7 except that butyl epoxy stearate was used as the epoxide reactant.                                                                             | 177                                             |
|         | 19          | A product prepared as in Example 2 except that the glycol used in the preparation of the phosphorodithioic acid was dipropylene glycol.                                           | 774                                             |
|         | 20          | A product prepared as in Example 5 except that the glycol used in the preparation of the phosphorodithioic acid was butyl epoxy stearate.                                         | 924                                             |
|         | 21          | A product prepared by the reaction of zinc di-(2-methylpentyl-4) phosphorodithioate with dodecene oxide.                                                                          | 330                                             |
|         | 22          | A product prepared as in Example 7 except that butylene oxide was the epoxide reactant.                                                                                           | 348                                             |

Other modes of applying the principle of the invention may be employed, change being made as regards the details described, provided the features stated in any of the following claims or the equivalent of such be employed.

I therefore particularly point out and distinctly claim as my invention:

1. The process of inhibiting corrosion of phosphated metal surfaces which comprises applying to said surfaces a film of a product prepared by the process which comprises the reaction of

(a) a zinc salt of a phosphorodithioic acid with (b) an approximately equivalent amount of an organic epoxide containing at least 4 aliphatic carbon atoms.

2. The process of claim 1 characterized further in that the phosphorodithioic acid of (a) is prepared by the reaction of phosphorus pentasulfide with a mixture of organic hydroxy compounds selected from the class consisting of alcohols and phenols.

3. The process of claim 1 characterized further in that the phosphorodithioic acid of (a) is prepared by the reaction of phosphorus pentasulfide with a mixture of aliphatic alcohols.

4. The process of claim 3 characterized further in that the mixture of alcohols is a mixture of a monohydric alcohol and a glycol.

5. The process of claim 3 characterized further in that the mixture of alcohols is a mixture of an octyl alcohol and a glycol.

6. The process of claim 3 characterized further in that the mixture of alcohols is a mixture of an octyl alcohol and dipropylene glycol.

7. The process of claim 1 characterized further in that the epoxide is an aliphatic epoxide.

8. The process of claim 1 characterized further in that the epoxide is an aliphatic epoxide containing 12-20 carbon atoms per epoxy group.

9. The process of inhibiting corrosion of phosphated metal surfaces which comprises applying to said surfaces a film of a product prepared by the process which comprises the reaction of

(a) a zinc salt of a phosphorodithioic acid prepared by the reaction of phosphorus pentasulfide with a mixture of a monohydric alcohol and a glycol with

(b) an approximately equivalent amount of an aliphatic

epoxide containing 12-20 carbon atoms per epoxy group.

10. The process of claim 9 characterized further in that the phosphorodithioic acid of (a) is prepared by the reaction of phosphorus pentasulfide with a mixture of equivalent amounts of an octyl alcohol and an aliphatic glycol.

11. The process of claim 9 characterized further in that the epoxide of (b) is butyl epoxy stearate.

References Cited in the file of this patent

UNITED STATES PATENTS

- |           |                 |               |
|-----------|-----------------|---------------|
| 2,063,629 | Salzberg et al. | Dec. 8, 1936  |
| 2,541,027 | Bradley         | Feb. 13, 1951 |
| 2,671,758 | Vinograd et al. | Mar. 9, 1954  |